

F. VON KÜGELGEN & G. O. SEWARD.

PRODUCTION OF MAGNESIUM.

APPLICATION FILED JULY 8, 1907.

935,796.

Patented Oct. 5, 1909.

FIG. 1.



FIG. 2.



INVENTORS:

Franz Von Kügelgen,  
and George O. Seward,

By Attorneys.

William G. Draper & Usina,

WITNESSES:

Fred White

Rene' Mune

# UNITED STATES PATENT OFFICE.

FRANZ VON KÜGELGEN, OF HOLCOMBS ROCK, VIRGINIA, AND GEORGE O. SEWARD, OF EAST ORANGE, NEW JERSEY, ASSIGNEES TO VIRGINIA LABORATORY COMPANY, OF NEW YORK, N. Y., A CORPORATION OF NEW YORK.

## PRODUCTION OF MAGNESIUM.

935,796.

Specification of Letters Patent.

Patented Oct. 5, 1909.

Application filed July 8, 1907. Serial No. 382,596.

To all whom it may concern:

Be it known that we, FRANZ VON KÜGELGEN, a subject of the German Emperor, residing at Holcombs Rock, in the county of 5 Bedford and State of Virginia, and GEORGE O. SEWARD, a citizen of the United States, residing at East Orange, in the county of Essex and State of New Jersey, have jointly invented certain new and useful Improvements 10 in the Production of Magnesium, of which the following is a specification.

The production of magnesium by the electrolysis of its molten chlorid is difficult for the reason that the specific gravity of the 15 electrolyte is very nearly the same as that of the metal and there are no fluxes which can be used to lower the specific gravity of the electrolyte sufficiently to insure a good separation of the metal therefrom.

Moreover, it is exceedingly difficult to 20 avoid the introduction of impurities such as iron when preparing the electrolyte, and such impurities,—being less electro-positive than magnesium and depositing together 25 with magnesium,—cause the formation of a spongy deposit of metal at the cathode which prevents the merging of the globules of magnesium.

The present invention provides a method 30 for the production of magnesium which overcomes the above-mentioned difficulties and which is characterized by being a process in two steps or operations. The first step produces an alloy of magnesium with a less 35 electro-positive metal by electrolyzing a molten magnesium electrolyte with an insoluble anode and a cathode of a molten metal, less electro-positive than magnesium. The second step produces pure magnesium by consecutive 40 dissolution and deposition from such alloy, the latter being used as the anode in a suitable electrolyte. In the first step any less electro-positive metals than magnesium, which may be present as impurities in 45 the initial electrolyte, are separated together with the magnesium and are absorbed by the molten alloy of the cathode. In the second step these impurities, being less electro-positive than magnesium, are not dissolved there- 50 with but remain in the molten anode; pure magnesium being thus produced. In the first step an electrolyte of low specific gravity is used so that an alloy very rich in magnesium can be produced without danger of

its leaving its position at the bottom of the 55 electrolytic vessel. In the second step an electrolyte is used of sufficiently high specific gravity to insure the rapid flotation of the magnesium to the surface as soon as deposited and its collection there. As a 60 cathode in the first step, we select a metal which (1) alloys easily with magnesium and forms a sufficiently fusible alloy therewith; (2) is capable of dissolving the impurities of the electrolyte which are less electro-positive than magnesium, and hence are deposited therewith; (3) is less electro-positive than magnesium so that, in the second step of the process, it remains unchanged while the magnesium dissolves in the electrolyte. 70 Aluminum combines these three properties and is a suitable metal for the cathode alloy.

In practicing our invention we proceed preferably as follows:—We subject a molten electrolyte of the approximate composition 75  $MgCl_2 + KCl$  to the action of a continuous electric current in a suitable vessel, using carbon anodes and a cathode of molten aluminum. The magnesium produced at the cathode alloys with the aluminum. As the 80 electrolysis proceeds the alloy becomes richer in magnesium; when it contains from 50 to 60 per cent. of magnesium it is removed either in whole or in part and is used as the anode in the second step of the process. 85

The electrolyte in the second step may be similar to that in the first step excepting that a certain proportion of a heavy salt of a more electro-positive metal than magnesium (e. g. barium-chlorid) is added to increase 90 the specific gravity and facilitates the flotation of the magnesium. As magnesium is dissolved from the anode to the same extent as it is deposited at the cathode, the electrolyte in the second step of the process remains substantially unchanged. Magnesium, being the most electro-positive constituent of the molten anode in the second step of the process, is alone dissolved and redeposited, care being taken to avoid exhausting the anode too much of its magnesium content. 95

In the accompanying drawings, Figure 1 is a vertical section of a suitable electrolytic cell for use in the first step of the process, and Fig. 2 is a similar section of a cell suitable for the second step. 100

Referring to Fig. 1, the electrolytic cell

or vessel A is shown as constructed with a receptacle C, which may be of cast metal, having a carbon lining D in its lower part and a water-jacket E surrounding its upper portion, whereby the electrolyte is chilled or incrusted to form a protective coating F. The vessel is covered by a top or lid G, which may be of graphite, and which is separated from the metal vessel below by an insulating layer H. Through the graphite top project one or more anodes J J which may be of graphite. These are connected to the positive terminal of the dynamo or other generator K, its negative terminal being connected to the vessel C or carbon lining D. A tap-hole L is provided through which to draw off the aluminum. An opening Q may be provided through the lid G for the escape of chlorin.

20 Referring to Fig. 2, the electrolytic cell or vessel B in which the second step of the process is performed, may be in general of somewhat similar construction to the vessel A. Its body or receptacle C' may be a duplicate of the vessel C, with a carbon lining D' and a water jacket E', forming a chilled layer of salt F' and having a tap-hole L'. The cover G' is here shown of cast metal separated from the vessel C' by insulation 30 H'. The cover has a flange I' projecting down beneath the surface of the electrolyte, so that it may serve initially as the cathode. It may also have a suitable lid M. The positive terminal of the generator K' is connected to the vessel C' or lining D', while its negative terminal is connected to the cover G'.

In operation, the alloy of magnesium and aluminum which is obtained in vessel A 40 is used as the anode in vessel B. After the second step has been in progress for a short time the separated magnesium covers the surface of the electrolyte and acts as the true cathode.

45 The operation in vessel A is made continuous by tapping off a part of the electrolyte from time to time and replacing it by exhausted alloy from the anode of vessel B.

The operation in vessel B is made continuous by removing a large part of the magnesium from time to time, and by tapping most of the nearly exhausted alloy of the anode from time to time and replacing by rich alloy from vessel A.

55 Though we have described the use of a chlorid electrolyte in both steps of our invention, we do not confine ourselves to such use, but may use any suitable electrolyte for either step of the process.

60 We are aware that impure aluminum has been purified by using it as the anode and dissolving it by electrolyzing with a solvent electrolyte, redepositing the resulting pure aluminum at the cathode. But we are not 65 aware that this process has been applied

with magnesium instead of aluminum. The conditions presenting difficulties in the production of magnesium by the electrolysis of its chlorid as hereinbefore stated, are different from those existing with aluminum.

70 By our invention we make as the first step of the process a suitable alloy of magnesium, solely in order that we may use this alloy as the anode in the final step of the process, from which to dissolve out therefrom the pure magnesium and collect it at the top of the electrolyte. We thus avoid the difficulty herein stated that in the direct production of magnesium from its molten chlorid the specific gravity of the electrolyte is so nearly that of the metal as to 75 impede the separation of the metal therefrom.

76 We claim as our invention:—

1. The process of obtaining magnesium which consists in producing an alloy of magnesium with a less electro-positive metal by electrolyzing a suitable electrolyte with a cathode of said metal; and subsequently dissolving the magnesium out of said alloy 85 by using the latter as an anode with a suitable molten electrolyte and depositing the magnesium at the cathode.

2. The process of obtaining magnesium which consists in electrolyzing a magnesium salt with a cathode of a metal less electro-positive than magnesium and which forms therewith an alloy of lower melting point; and subsequently dissolving the magnesium out of said alloy by using the latter as an 90 anode with a suitable molten electrolyte and depositing the magnesium at the cathode.

3. The process of obtaining magnesium which consists in electrolyzing fused magnesium chlorid with a cathode of a metal less electro-positive than magnesium to form an alloy therewith; and subsequently dissolving the magnesium out of said alloy by using the latter as an anode with a suitable molten electrolyte and depositing the magnesium at the cathode.

105 4. The process of obtaining magnesium which consists in electrolyzing a magnesium salt with a cathode of molten aluminum to produce a magnesium-aluminum alloy; and subsequently dissolving the magnesium out of said alloy by using the latter as an anode with a suitable molten electrolyte and depositing the magnesium at the cathode.

110 5. The process of obtaining magnesium which consists in electrolyzing a magnesium salt with a cathode of molten magnesium-aluminum alloy thereby adding magnesium to such alloy; and subsequently dissolving the magnesium out of said alloy and using the latter as an anode with a suitable molten electrolyte and depositing the magnesium at the cathode.

120 6. The process of obtaining magnesium which consists in electrolyzing magnesium

76

75

80

90

95

100

105

110

115

120

125

130

chlorid with a cathode of molten aluminum to form a magnesium-aluminum alloy; and subsequently dissolving the magnesium out of said alloy by using the latter as an anode 5 with an electrolyte of magnesium chlorid to which is added a heavy salt of a more electro-positive metal to increase its specific gravity, whereby the magnesium separated at the cathode is caused to float upon the 10 electrolyte.

7. In the process of obtaining magnesium by first electrically producing an alloy thereof with another metal, the step of recovering the magnesium from said alloy which consists in electrolyzing an electrolyte of a mag- 15

nesium salt to which a heavy salt of a more electro-positive metal has been added to increase its specific gravity, using said alloy as the anode whereby magnesium is dissolved out therefrom and deposited at the 20 cathode, and the separated magnesium is caused to float upon said electrolyte.

In witness whereof, we have hereunto signed our names in the presence of two subscribing witnesses.

FRANZ VON KÜGELGEN.  
GEORGE O. SEWARD.

Witnesses:

HARRY R. LEE,  
J. H. WEBB.